



US005965333A

# United States Patent [19]

Chen et al.

[11] Patent Number: 5,965,333

[45] Date of Patent: Oct. 12, 1999

[54] THERMAL RECORDING ELEMENT

[56]

**References Cited**[75] Inventors: **Huijuan D. Chen, Webster; Derek D. Chapman; Margaret J. Helber**, both of Rochester, all of N.Y.**U.S. PATENT DOCUMENTS**3,247,127 4/1966 Bailly .  
4,767,696 8/1988 Ishimoto et al. .... 430/495[73] Assignee: **Eastman Kodak Company**, Rochester, N.Y.*Primary Examiner*—Thorl Chea  
*Attorney, Agent, or Firm*—Harold E. Cole

[21] Appl. No.: 09/037,206

**ABSTRACT**

[22] Filed: Mar. 10, 1998

A thermal recording element comprising a support having thereon a recording layer comprising a J-aggregate derived from an oxonol dye dispersed in a hydrophilic binder.

[51] Int. Cl.<sup>6</sup> G03C 1/72; G03C 5/16**20 Claims, No Drawings**[52] U.S. Cl. 430/351; 430/19; 430/495.1;  
430/944; 430/945; 346/135.1[58] Field of Search 430/19, 17, 945,  
430/495.1, 944, 270.18, 292, 351; 346/135.1

1

## **THERMAL RECORDING ELEMENT**

## FIELD OF THE INVENTION

This invention relates to thermal recording elements, and more particularly to such elements which contain a J-aggregate dye derived from an oxonol for generating visual continuous tone images in a single-sheet process.

## BACKGROUND OF THE INVENTION

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to one of the cyan, magenta or yellow signals. The process is then repeated for the other two colors. A color hard copy is thus obtained which corresponds to the original picture viewed on a screen. Further details of this process and an apparatus for carrying it out are contained in U.S. Pat. No. 4,621,271, the disclosure of which is hereby incorporated by reference.

Another way to thermally obtain a print using the electronic signals described above is to use a laser instead of a thermal printing head. In such a system, the donor sheet includes a material which strongly absorbs at the wavelength of the laser. When the donor is irradiated, this absorbing material converts light energy to thermal energy and transfers the heat to the dye in the immediate vicinity, thereby heating the dye to its vaporization temperature for transfer to the receiver. The absorbing material may be present in a layer beneath the dye and/or it may be admixed with the dye. The laser beam is modulated by electronic signals which are representative of the shape and color of the original image, so that each dye is heated to cause volatilization only in those areas in which its presence is required on the receiver to reconstruct the color of the original object. Further details of this process are found in GB 2,083,726A, the disclosure of which is hereby incorporated by reference.

Still another way to generate an image in a thermal recording process is to use a direct thermal recording element which contains a material which, when heated with a thermal head or an infrared laser, forms a visible image. In this process, there is no transfer of dye to a separate receiving element.

## DESCRIPTION OF RELATED ART

U.S. Pat. No. 4,767,696 relates to a laser information recording system comprising a substrate, a reflective layer, and a recording layer. The recording layer comprises cumulative sublayers of J-aggregate dyes formed from mixtures of a cyanine dye and at least two specific cationic film-forming materials using the Langmuir-Blodgett thin film technique.

When organic dye molecules, e.g., oxonol dye molecules, are highly concentrated in an aqueous solution, there

2

appears an absorption band or peak which has a large absorption intensity at a longer wavelength than is the case of a single molecule absorption band and has a very narrow half-amplitude level. This absorption band is called the J-absorption band and is known to derive from aggregates of dye molecules called J-aggregates. J-aggregates are characterized by a narrow intense absorption peak that is bathochromically shifted relative to the monomer absorption.

However, there is a problem with using these J-aggregates in a thermal recording layer in that the efficiency of deaggregation is low, causing very poor contrast, as will be shown hereinafter.

It is an object of this invention to provide a thermal recording element using a J-aggregate which has a high deaggregation efficiency. It is another object of the invention to provide a thermal recording element using a J-aggregate which has high image contrast to give a visual continuous tone upon imagewise heating.

## SUMMARY OF THE INVENTION

These and other objects are achieved in accordance with this invention which relates to a thermal recording element comprising a support having thereon a recording layer a 25 J-aggregate derived from an oxonol dye dispersed in a hydrophilic binder.

## DESCRIPTION OF THE PREFERRED EMBODIMENTS

30 The present invention uses a single-layer coating containing a J-aggregate oxonol dye in a hydrophilic polymer binder, such as gelatin, and generates visual images by imagewise heating of this single layer. The oxonol dyes readily form J-aggregates in a gelatin coating without additional film-forming materials when such a coating dries on a substrate. The element is easy to coat and its structure is 35 simple, having only the recording layer on a support.

The J-aggregate dyes employed in the invention have sharp absorption peaks that are bathochromically shifted relative to their nonaggregated states when these dyes are coated in a hydrophilic binder such as gelatin. When heated with a thermal head, flash or an infrared laser, a visible image with high contrast ( $D_{max}/D_{min}$  up to 10) can be generated due to deaggregation of the dye aggregate.

45 In a preferred embodiment of the invention, the J-aggregate dye employed in the invention is derived from a barbituric acid oxonol having the formula:



12. wherein:

each X independently represents O or S:

$R^1$ ,  $R^2$ ,  $R^3$  and  $R^4$  each independently represents hydrogen, a substituted or unsubstituted alkyl or alkoxy group having from about 1 to about 6 carbon atoms, such as methyl, ethyl, propyl, methoxyethyl, methoxy, ethoxy, etc.; a substituted or unsubstituted aryl group having from about 6 to about 10 atoms, such as phenyl,

tolyl, etc.; or a substituted or unsubstituted heteroaryl group having from about 5 to about 10 atoms, such as pyrrolo;

$L^1$ ,  $L^2$  and  $L^3$  each independently represents a substituted or unsubstituted methine group;

$M^+$  represents a proton or an inorganic or organic cation, such as triethylammonium, potassium, sodium; and  $n$  is 0-3.

Examples of J-aggregates derived from an oxonol dye employed in the invention are as follows:

TABLE 1

| Dye    | $R^{13}$ | $R^{14}$ | $R^{15}$ | $R^{16}$ | $R^{17}$ | $M^+$          |
|--------|----------|----------|----------|----------|----------|----------------|
|        |          |          |          |          |          |                |
| 1 (a)  | H        | H        | $OCH_3$  | H        | $CH_3$   | H              |
| 1 (b)  | H        | H        | $OCH_3$  | H        | $CH_3$   | $(C_2H_5)_3NH$ |
| 2      | H        | H        | OH       | H        | $CH_3$   | H              |
| 3      | H        | H        | $CH_3$   | H        | $CH_3$   | H              |
| 4      | H        | H        | $OCH_3$  | H        | $C_2H_5$ | H              |
| 5 (a)  | H        | H        | H        | $OCH_3$  | $CH_3$   | H              |
| 5 (b)  | H        | H        | H        | $OCH_3$  | $CH_3$   | Na             |
| 6 (a)  | H        | $OCH_3$  | H        | H        | H        | H              |
| 6 (b)  | H        | $OCH_3$  | H        | H        | H        | $(C_2H_5)_3NH$ |
| 7      | $OCH_3$  | H        | H        | H        | H        | H              |
| 8 (a)  | H        | H        | OH       | H        | H        | H              |
| 8 (b)  | H        | H        | OH       | H        | H        | $(C_2H_5)_3NH$ |
| 9      | H        | H        | OH       | H        | H        | PyrH*          |
| 10 (a) | H        | OH       | H        | H        | H        | H              |
| 10 (b) | H        | OH       | H        | H        | H        | PyrH           |
| 11     | H        | $CH_3$   | H        | H        | H        | H              |
| 12     | H        | $CONH_2$ | H        | H        | H        | H              |
| 13     | H        | H        | H        | H        | H        | H              |
| 14     | H        | H        | H        | H        | $CH_3$   | H              |
| 15     | H        | $CH_3$   | H        | H        | $CH_3$   | H              |
| 16     | H        | $COOH$   | H        | H        | $CH_3$   | H              |
| 17     | H        | Cl       | H        | Cl       | H        | H              |
| 18     | $OCH_3$  | $OCH_3$  | H        | H        | H        | H              |
| 19     | H        | $OCH_3$  | H        | $OCH_3$  | H        | H              |
| 20     | H        | $OCH_3$  | $CH_3$   | H        | H        | H              |
| 21     | H        | OH       | OH       | H        | H        | H              |

\*PyrH designates a protonated pyridinium group

TABLE 2

| Dye    | $R^{13}$ | $R^{14}$ | $R^{15}$     | $R^{16}$ | $M^+$          |
|--------|----------|----------|--------------|----------|----------------|
|        |          |          |              |          |                |
| 22 (a) | H        | OH       | H            | H        | H              |
| 22 (b) | H        | OH       | H            | H        | PyrH           |
| 23     | H        | H        | OH           | H        | H              |
| 24     | H        | H        | $NHSO_2CH_3$ | H        | $(C_2H_5)_3NH$ |
| 25     | H        | H        | $COOH$       | H        | H              |
| 26     | OH       | H        | H            | H        | H              |

In another preferred embodiment of the invention, the J-aggregate a barbituric acid oxonol dye employed in the invention has the formula:



wherein

R represents a hydrogen atom or substituted or unsubstituted alkyl, aryl or acyl group; and R<sup>1</sup>, R<sup>2</sup>, R<sup>3</sup>, R<sup>4</sup> and M<sup>+</sup> are the same as in formula (I).

In another preferred embodiment of the invention, the J-aggregate derived from a barbituric acid oxonol dye employed in the invention has the formula:



wherein

R represents a hydrogen atom or substituted or unsubstituted alkyl, aryl or acyl group; and R<sup>1</sup>, R<sup>2</sup>, R<sup>3</sup>, R<sup>4</sup> and M<sup>+</sup> are the same as in formula (I).

In another preferred embodiment, the J-aggregate dye employed in the invention is derived from a benzothiophene dioxide oxonol having the formula:



wherein:

R<sup>5</sup>–R<sup>12</sup> each independently represent an unsubstituted or substituted alkyl group, an unsubstituted or substituted aryl group or an unsubstituted or substituted heteroaryl group, a hydrogen atom, halogen, for example, chloro, fluoro, bromo, iodo; alkoxy, aryloxy, carbonamido, carbamoyl, substituted or unsubstituted amino group, an acyl group, a carboxylic acid group, a substituted or unsubstituted thio group, a hydroxyl group, a sulfonamido group, a nitro group, a cyano group, a sulfonic acid group, a sulfamoyl group; or adjacent pairs of substituents represented by R<sup>5</sup>–R<sup>12</sup> may form a fused 5- or 6-membered substituted or unsubstituted aromatic or heteroaromatic ring;

L<sup>4</sup>, L<sup>5</sup> and L<sup>6</sup> each independently represents substituted or unsubstituted methine group, M<sup>+</sup> represents a proton or an inorganic or organic cation; and

m is 0, 1, 2, or 3.

Examples of preferred benzothiophene dioxide oxonols employed in the invention are shown in the following Table 3.

TABLE 3

| Dye | m | R<sup>5</sup> and R<sup>9</sup> |               | R<sup>6</sup> and R<sup>10</sup> |                | R<sup>7</sup> and R<sup>11</sup> |                | R<sup>8</sup> and R<sup>12</sup> |                |
|-----|---|---------------------------------|---------------|----------------------------------|----------------|----------------------------------|----------------|----------------------------------|----------------|
|     |   | R<sup>5</sup>                   | R<sup>9</sup> | R<sup>6</sup>                    | R<sup>10</sup> | R<sup>7</sup>                    | R<sup>11</sup> | R<sup>8</sup>                    | R<sup>12</sup> |
| 27  | 1 | H                               |               | H                                |                | Cl                               |                | H                                |                |
| 28  | 1 | H                               |               | OCH<sub>3</sub>                  |                | H                                |                | H                                |                |
| 29  | 1 | H                               |               | CH<sub>3</sub>                   |                | H                                |                | H                                |                |
| 30  | 0 | H                               |               | H                                |                | F                                |                | H                                |                |
| 31  | 0 | H                               |               | H                                |                | Cl                               |                | H                                |                |
| 32  | 0 | Cl                              |               | H                                |                | H                                |                | Cl                               |                |
| 33  | 0 | H                               |               | CH<sub>3</sub>                   |                | H                                |                | H                                |                |
| 34  | 0 | H                               |               | OCH<sub>3</sub>                  |                | H                                |                | H                                |                |

Another embodiment of the invention relates to a process of forming a single color image comprising imagewise-exposing by means of a flash, thermal print head or laser, in the absence of a separate receiving element, the thermal recording element as described above, thereby imagewise-heating the recording layer and causing it to change color, thereby creating the single color image.

To prepare the recording layer coating of the invention, the chosen oxonol dye is added in the form of a solid particle dispersion (SPD) to an aqueous medium comprising water and a hydrophilic binder, such as gelatin (preferably deionized gelatin). The solid particle dispersion comprising solid microcrystalline particles of a dye can be prepared by forming a slurry of the dye in an aqueous medium comprising water and a surfactant and then subjecting the slurry to a milling procedure, such as ball-milling, sand-milling, media-milling or colloid-milling. The coating melt can then be subjected to heat treatment at elevated temperatures, such as 40° C.–100° C., for a period of time, such as 5 min to 24 hrs. Adjustments of the pH and ionic strength of the melt may be necessary to control dye solubility in the aqueous medium. Typically, the dye concentration in the melt is 0.05%–1%, by weight, at a laydown of 0.02–0.16 g/m<sup>2</sup>; and the gelatin concentration in the melt is 0.88%–6.6%, by weight, with a laydown of 0.22–1.62 g/m<sup>2</sup>.

Different methods of heating can be used to image the thermal recording elements of the invention. For example, a flash can be used such as a xenon flash lamp with a maximum energy of 9 J/cm<sup>2</sup>. A thermal print head can also be used such as one with a heating voltage of 12–14 v and a heating speed of 4 ms/line for a 640 line image. Further, an infrared laser writer can be used such as Laser Model SDL-2420-H2 from Spectra Diode Labs, or Laser Model SLD 304 V/W from Sony Corp.

The recording elements of this invention can be used to obtain medical images, reprographic masks, printing masks, etc. The image obtained can be a positive or a negative image. The process of the invention can generate either continuous (photographic-like) or halftone images.

Any hydrophilic material may be used as the binder in the recording element employed in the invention. For example, there may be used gelatin, a poly(ethylene oxide), a poly(vinyl alcohol), a polyacrylic acid, a poly(vinyl

pyrrolidone), poly(vinylpyridine), poly(hydroxyethyl acrylate) or mixtures or copolymers thereof. The binder may be used at a coverage of from about 0.1 to about 5 g/m<sup>2</sup>.

When the absorption in the IR region of the J-aggregate dye is not sufficient for IR laser imaging, then an additional water-soluble IR absorber may be used. Such water-soluble infrared-absorbing materials include cyanine infrared-absorbing dyes as described in U.S. Pat. No. 5,695,918, the disclosure of which is hereby incorporated by reference. The infrared-absorbing material may be either in the recording layer or a layer underneath or on top thereof.

C) An element similar to A) was prepared except that Dye 3 was employed instead of Dye 1(a).

D) An element similar to A) was prepared except that Dye 22(a) was employed instead of Dye 1(a).

E) An element similar to A) was prepared except that Dye 27 was employed instead of Dye 1(a).

10 Control) A control element similar to A) was prepared except that C-1, a cyanine dye from U.S. Pat. No. 4,769,696, was employed instead of Dye 1(a):



Any material can be used as the support for the recording element of the invention provided it is dimensionally stable and can withstand the heat of the flash, thermal head or laser. Such materials include polyesters such as poly(ethylene naphthalate); polysulfones; poly(ethylene terephthalate); polyamides; polycarbonates; cellulose esters such as cellulose acetate; fluorine polymers such as poly(vinylidene fluoride) or poly(tetrafluoroethylene-co-hexafluoropropylene); polyethers such as polyoxymethylene; polyacetals; polyolefins such as polystyrene, polyethylene, polypropylene or methylpentene polymers; and polyimides such as polyimide-amides and polyether-imides. The support generally has a thickness of from about 5 to about 200  $\mu$ m. It can be transparent or opaque such as paper.

The following examples are provided to illustrate the invention.

## EXAMPLES

### Example 1

#### Flash Exposure

A) A solid particle dispersion of a barbituric acid oxonol Dye 1(a) was prepared based on the media-milling method. The slurry containing 0.75 g Dye 1(a), 0.75 g 10% polyvinylpyrrolidone (PVP) aqueous solution, 13.5 g doubly distilled water, and 21.0 mL media beads (0.6–0.8 mm in diameter) was milled at a speed of 2000 rpm for 4 hours at pH<5.0 using a micromilling apparatus. The solid particle dispersion was collected by filtering the mixture with a stainless steel screen to remove the media beads.

A suitable amount of the above solid particle dispersion was added to the melt of gelatin (deionized) so that the final concentrations of Dye 1(a) and gelatin in the melt were 0.22% wt-% and 2.2 wt-%, respectively. The solution was heated to 50° C. for 30 min. and then coated onto a poly(ethylene terephthalate) support with a final laydown of 0.05 g/m<sup>2</sup> of dye and 0.54 g/m<sup>2</sup> of gelatin. The coating was chill-set and allowed to air-dry overnight before the imaging experiment was run.

B) An element similar to A) was prepared except that Dye 2 was employed instead of Dye 1(a).

25 The  $\lambda$ -max of the dyes used in the above elements was measured using a Hewlett-Packard 8453 diode array spectrophotometer in transmission mode.

30 The element was then imaged by subjecting it to a flash lamp exposure. The window of a flash lamp capable of delivering 9 joules/cm<sup>2</sup> was fitted with a mirror box that reduced the exit aperture to 11×14 cm. On top of this was placed a mask having an aperture of 1.2×4.2 cm. The element was then placed in contact with the mask and covered with a piece of white paper and a glass plate. The flash was fired at full intensity, the element removed and the visible spectrum measured with the above spectrophotometer.

35 Dark stability testing of the imaged samples was then performed in a wet oven at 50° C., 50% RH for 5 days, and the stability was evaluated based on the percent loss of the absorption maxima of the imaged and nonimaged samples. The results are also shown in the following Table 4:

45

TABLE 4

| 50    | Dye | CH <sub>3</sub> OH | Coated | flash | λ-max |      | D-min | Dark Stability (%) |        |
|-------|-----|--------------------|--------|-------|-------|------|-------|--------------------|--------|
|       |     |                    |        |       | (nm)  | (nm) |       | As Coated          | Imaged |
| 1(a)  |     | 611                | 790    | 621   | 169   | 10.0 | 621   | -2.9%              | -1.7%  |
| 2     |     | 609                | 780    | 623   | 157   | 3.7  | 623   | 0.0%               | +7.0   |
| 3     |     | 609                | 784    | 622   | 162   | 3.25 | 622   | 0.0%               | +1.6%  |
| 22(a) |     | 488                | 558    | 490   | 68    | 4.4  | 490   | -1.1%              | -0.3%  |
| 27    |     | 551                | 610    | 562   | 48    | 3.6  | 562   | -2.7%              | +0.4%  |
| C-1   |     | 659                | 730    | 673   | 57    | 1.8  | 673   | -3.0%              | -2.2%  |

60 The above results show that a significant color change was observed for all the examples upon flash exposure. In the elements containing Dyes 1(a), 2 and 3, a cyan image was generated on a near colorless background due to the formation of a J-aggregate in the near infrared region ( $\lambda$ .max $\geq$ 780 nm). All the examples except the control show a reasonable D-max/D-min value (>3.0).

65 The cyanine dye from U.S. Pat. No. 4,767,696 (the control) forms a broad J-aggregate at 730 nm under the experimental conditions of the current invention as com-

pared with the J-aggregate formation at 780 nm in the presence of cationic film forming materials shown in U.S. Pat. No. 4,767,696. However, this dye only showed a moderate image contrast ( $D_{max}/D_{min}=1.8$ ) and a high background due to aggregation closer to the visible region of the spectrum with a  $\lambda_{max}$  at 730 nm. These imaging samples also show good dark stability.

### Example 2

#### Thermal Print Head Exposure

The elements of Example 1 were imaged with a thermal resistive head in a stepwise fashion at a heating speed of 4 ms/line for a 640 line image and heating voltage of 14 v.

The imaging electronics were activated causing the element to be drawn through the printing head/roller nip at 40.3 mm/sec. Coincidentally, the resistive elements in the thermal print head were pulsed for 127.75  $\mu$ s/pulse at 130.75  $\mu$ s intervals during a 4.575 ms/dot printing cycle (including a 0.391 ms/dot cool down interval). A stepped image density was generated by incrementally increasing the number of pulses/dot from a minimum of 0 to a maximum of 32 pulses/dot. The voltage supplied to the thermal head was approximately 14.0 v resulting in an instantaneous peak power of 0.369 watts/dot and a maximum total energy of 1.51 mJ/dot; print room humidity: 42–45% RH. The following images were obtained on a light-blue background except for element C where a magenta image was obtained on a blue background:

TABLE 5

| Element | Dye  | $\lambda_{max}(\text{nm})$<br>as Coated | $\lambda_{max}(\text{nm})$<br>After Printing | $\Delta\lambda(\text{nm})$ | $D_{max}/D_{min}$ |
|---------|------|-----------------------------------------|----------------------------------------------|----------------------------|-------------------|
| A       | 1(a) | 790                                     | 621                                          | 169                        | 6.6               |
| B       | 2    | 780                                     | 622                                          | 158                        | 3.0               |
| C       | 3    | 784                                     | 622                                          | 162                        | 4.4               |
| Control | C-1  | 730                                     | 673                                          | 57                         | 1.5               |

The above results show that similar color change was observed for thermal print head exposure as compared to flash lamp exposure with slightly lower  $D_{max}/D_{min}$ . In the elements containing Dyes 1(a), 2, 3 and C-1, a 640 line cyan digital image was obtained. Again, the control dye C-1 gives the lowest  $D_{max}/D_{min}$  value.

### Example 3

#### Laser Exposure

A) Element A of Example 1 was employed except that it contained the following IR absorber in an amount of 0.22 wt-% so as to give a final laydown of 0.05 g/m<sup>2</sup> of IR Absorber dye:



The element was imaged with an IR laser writer (830 nm) with maximum energy of 300 mJ/cm<sup>2</sup>.

Control) A control element similar to the Control of Example 1 was employed except that it contained the IR absorber of A) in an amount of 0.22 wt-% so as to give a final laydown of 0.05 g/m<sup>2</sup> of the IR Absorber dye.

The above elements were written using a laser diode print head, where each laser beam has a wavelength range of 830–840 nm and a nominal power output of 600 mW at the film plane. The drum, 53 cm in circumference was rotated at varying speeds and the imaging electronics were activated to provide adequate exposure. The translation stage was incrementally advanced across the recording element by means of a lead screw turned by a microstepping motor, to give a center-to-center line distance of 10.58  $\mu$ m (945 lines per centimeter or 2400 lines per inch). The measured total power at the focal plane was 600 mW per channel. At a rotation of 1000 rpm, the exposure was about 300 mJ/cm<sup>2</sup>. The following results were obtained:

TABLE 6

| Element | Dye  | $\lambda_{max}(\text{nm})$<br>as Coated | $\lambda_{max}(\text{nm})$<br>After Printing | $\Delta\lambda(\text{nm})$ | $D_{max}/D_{min}$ |
|---------|------|-----------------------------------------|----------------------------------------------|----------------------------|-------------------|
| A       | 1(a) | 790                                     | 621                                          | 169                        | 9.6               |
| Control | C-1  | 730                                     | 673                                          | 57                         | 1.8               |

The above results show that the above elements can be imaged with laser writer similar to flash exposure and thermal resistive head printing. A cyan digital image was obtained for Dye 1(a) and the control. The  $D_{max}/D_{min}$  value for laser imaging is close to that of the flash exposure method.

The invention has been described in detail with particular reference to preferred embodiments thereof, but it will be understood that variations and modifications can be effected within the spirit and scope of the invention.

What is claimed is:

1. A thermal recording element comprising a support having thereon a single recording layer comprising a J-aggregate derived from an oxonol dye dispersed in a hydrophilic binder.

2. The recording element of claim 1 wherein said J-aggregate is derived from a barbituric acid oxonol dye having the formula:



wherein:

each X independently represents O or S;

$R^1$ ,  $R^2$ ,  $R^3$  and  $R^4$  each independently represents hydrogen, a substituted or unsubstituted alkyl group of from about 1 to about 6 carbon atoms, a substituted or unsubstituted aryl group having from about 6 to about 10 atoms or a substituted or unsubstituted heteroaryl group having from about 5 to about 10 atoms;

$L^1$ ,  $L^2$  and  $L^3$  each independently represents a substituted or unsubstituted methine group;

$M^+$  represents a proton or an inorganic or organic cation; and

$n$  is 0–3.

3. The recording element of claim 2 wherein said J-aggregate derived from a barbituric acid oxonol dye has the formula:

11



wherein R represents a hydrogen atom or a substituted or unsubstituted alkyl, aryl or acyl group; and R<sup>1</sup>, R<sup>2</sup>, R<sup>3</sup>, R<sup>4</sup> and M<sup>+</sup> are the same as in claim 2.

4. The recording element of claim 3 wherein each of R<sup>3</sup> and R<sup>4</sup> represents a hydrogen atom. 15

5. The recording element of claim 3 wherein R represents a hydrogen atom, a methyl or ethyl group.

6. The recording element of claim 2 wherein said dye has the formula: 20



wherein R represents a hydrogen atom or a substituted or unsubstituted alkyl, aryl or acyl group; and R<sup>1</sup>, R<sup>2</sup>, R<sup>3</sup>, R<sup>4</sup> and M<sup>+</sup> are the same as in claim 2.

7. The recording element of claim 6 wherein each of R<sup>3</sup> and R<sup>4</sup> represents a hydrogen atom. 25

8. The recording element of claim 1 wherein said J-aggregate is derived from a benzothienone dioxide oxonol dye having the formula: 30



wherein:

R<sup>5</sup>–R<sup>12</sup> each independently represents a substituted or unsubstituted alkyl, aryl or heteroaryl group, hydrogen, halogen, alkoxy, aryloxy, carbonamido, carbamoyl, substituted or unsubstituted amino group, acyl, carboxylic acid, substituted or unsubstituted thio, hydroxyl, sulfonamido, nitro, cyano, sulfonic acid, or sulfamoyl; 55

or adjacent pairs of substituents represented by R<sup>5</sup>–R<sup>12</sup> may form a fused 5- or 6-membered substituted or unsubstituted aromatic or heteroaromatic ring; 60

L<sup>4</sup>, L<sup>5</sup> and L<sup>6</sup> each independently represents a substituted or unsubstituted methine group;

M<sup>+</sup> represents a proton or an inorganic or organic cation; 65

and

m is 0 to 3.

12

9. The element of claim 8 wherein said J-aggregate is derived from a benzothienone dioxide oxonol dye having the formula:



wherein:

R<sup>5</sup>–R<sup>12</sup> and M<sup>+</sup> are the same as in claim 8.

10. The element of claim 1 wherein said recording layer has a water-soluble infrared-absorbing material associated therewith.

11. The element of claim 1 wherein said hydrophilic binder is gelatin.

12. A process of forming a single color image comprising imagewise-exposing by means of a flash, thermal print head or laser, in the absence of a separate receiving element, a thermal recording element comprising a support having thereon a single recording layer, thereby imagewise-heating said recording layer and causing it to change color to create said single color image, said recording layer comprising a J-aggregate derived from an oxonol dye dispersed in a hydrophilic binder.

13. The process of claim 12 wherein said J-aggregate is derived from a barbituric acid oxonol dye having the formula:



50 wherein:

each X independently represents O or S;

R<sup>1</sup>, R<sup>2</sup>, R<sup>3</sup> and R<sup>4</sup> each independently represents hydrogen, a substituted or unsubstituted alkyl group of from about 1 to about 6 carbon atoms, a substituted or unsubstituted aryl group having from about 6 to about 10 atoms or a substituted or unsubstituted heteroaryl group having from about 5 to about 10 atoms;

L<sup>1</sup>, L<sup>2</sup> and L<sup>3</sup> each independently represents a substituted or unsubstituted methine group;

M<sup>+</sup> represents a proton or an inorganic or organic cation; and

n is 0–3.

14. The process of claim 13 wherein said J-aggregate derived from a barbituric acid oxonol dye has the formula:

13



(II)

14



(IV)

wherein R represents a hydrogen atom or a substituted or unsubstituted alkyl, aryl or acyl group; and R<sup>1</sup>, R<sup>2</sup>, R<sup>3</sup>, R<sup>4</sup> and M<sup>+</sup> are the same as in claim 13.

15. The process of claim 14 wherein each of R<sup>3</sup> and R<sup>4</sup> represents a hydrogen atom.

16. The process of claim 14 wherein R represents a hydrogen atom, a methyl or ethyl group.

17. The process of claim 13 wherein said dye has the formula:



(III)

wherein R represents a hydrogen atom or a substituted or unsubstituted alkyl, aryl or acyl group; and R<sup>1</sup>, R<sup>2</sup>, R<sup>3</sup>, R<sup>4</sup> and M<sup>+</sup> are the same as in claim 13.

18. The process of claim 17 wherein each of R<sup>3</sup> and R<sup>4</sup> represents a hydrogen atom.

19. The process of claim 12 wherein said J-aggregate is derived from a benzothienone dioxide oxonol dye having the formula:

wherein:

R<sup>5</sup>-R<sup>12</sup> each independently represents a substituted or unsubstituted alkyl, aryl or heteroaryl group, hydrogen, halogen, alkoxy, aryloxy, carbonamido, carbamoyl, substituted or unsubstituted amino group, acyl, carboxylic acid, substituted or unsubstituted thio, hydroxyl, sulfonamido, nitro, cyano, sulfonic acid, or sulfamoyl; or adjacent pairs of substituents represented by R<sup>5</sup>-R<sup>12</sup> may form a fused 5- or 6-membered substituted or unsubstituted aromatic or heteroaromatic ring; L<sup>4</sup>, L<sup>5</sup> and L<sup>6</sup> each independently represents a substituted or unsubstituted methine group; M<sup>+</sup> represents a proton or an inorganic or organic cation; and m is 0 to 3.

20. The process of claim 19 wherein said J-aggregate is derived from a benzothienone dioxide oxonol dye having the formula:



(V)

wherein:

R<sup>5</sup>-R<sup>12</sup> and M<sup>+</sup> are the same as in claim 19.

\* \* \* \* \*